

United States Patent [19]  
Hager

[11] 3,865,932  
[45] Feb. 11, 1975

[54] COMPOUNDS OF COPPER, CHROMIUM  
AND ARSENIC AS WOOD PRESERVATIVES

[75] Inventor: **Bror Olof Hager, Djursholm,  
Sweden**

[73] Assignee: **Hager Aktiebolag, Stockholm SV,  
Sweden**

[22] Filed: **June 15, 1971**

[21] Appl. No.: **153,412**

**Related U.S. Application Data**

[63] Continuation of Ser. No. 733,825, June 3, 1968,  
abandoned.

[52] U.S. Cl. .... **424/128, 424/137**

[51] Int. Cl. .... **A01n 11/00**

[58] Field of Search..... **424/137, 128, 141**

[56]

**References Cited**

**FOREIGN PATENTS OR APPLICATIONS**

|         |         |                |         |
|---------|---------|----------------|---------|
| 27,826  | 12/1955 | Finland        |         |
| 102,457 | 11/1937 | Australia..... | 424/137 |
| 166,413 | 1/1956  | Australia..... | 424/137 |

*Primary Examiner*—Vincent D. Turner  
*Attorney, Agent, or Firm*—Pierce, Scheffler & Parker

[57]

**ABSTRACT**

The content of arsenic in conventional  $\text{MeO}-\text{CrO}_3-\text{As}_2\text{O}_5$  wood preservatives is partially replaced by phosphoric or sulfuric acid.

**3 Claims, No Drawings**

## COMPOUNDS OF COPPER, CHROMIUM AND ARSENIC AS WOOD PRESERVATIVES

This application is a continuation of my parent patent application Ser. No. 733,825 filed June 3, 1968, which parent application is now abandoned.

This invention relates to the wood preservation art, and is concerned with the provision of improved preservative compositions.

Aqueous solutions containing compounds of copper and chromium have long been used as wood preservatives. The copper compound usually has been copper sulphate, and the conserving effect of the preservative has mainly been based on the copper radical in this compound. The chromium compound has been a water-soluble chromate having the property of protecting ferrous metal impregnating apparatus against corrosion from the copper compound. Furthermore the chromate was observed to have the uniquely important property of fixing the copper compound in situ in the wood in an insoluble condition so that the copper could not be leached when the wood later was exposed to water or moisture. This fixation depended on the reduction of the chromate in contact with the wood, chromium radical hereby being converted from the six-valent negative, to a three-valent, positive, radical. Thus the chromium in the preservative is present as a negative, strong acid radical (ion) (i.e., chromic acid). As an acid it acts as a dissolving agent with respect to the different compounds in the preservative. The dissolving effect of the chromium compound ceases completely upon its reduction as noted above.

To this effect will be added the precipitating effect of the formed three-valent (basic) chromium radical. The same can neutralize other dissolving acid radicals such, for example, as sulphuric acid. In other cases the positive chromium can form difficultly soluble compounds. This happens when the said preservatives are combined with arsenic compounds, e.g., with arsenic acid or arsenates. When the positive three-valent chromium radical is formed in the wood the arsenic is precipitated wholly or partly as very difficultly soluble chromium arsenates.

A preservative (developed by applicant) which has been used to a large extent in different countries is based on these experiences. The dissolving effect of the chromium and arsenic acids has here been rationally utilized for dissolving the copper compound in the preservative, with very good fixation of the ingredients of the preservative in situ having been realized. This has occurred without forming injurious, soluble, non-conserving products in the wood, for instance, sodium sulphate. This preservative is described in Swedish Pat. No. 139,177 and 143,080 and in U.S. Pat. Nos. 2,432,007 and 2,565,175. In the last-mentioned patent the claims were directed to a method for manufacturing the preservative but in the specification the limits for the composition of the preservative are given. The preservative is also described in various foreign patents including Finnish Patents 25,857 — published in March 1949 — and 27,826, both with priority from 1946. In the latter of these Finnish patents the preservative was described with closer limits, the composition of the preservative being stated to be:



where Me represents a two-valent metal capable of forming difficultly soluble arsenates. Furthermore, the

following formula has been given showing the most suitable composition of the preservative:



5 If copper (Cu) is introduced where "Me" is written the exact composition is received of the above said preservative used in practice to a large extent in many different countries.

During the years this preservative has been used 10 many experiences and investigations have given impetus for further development. A first question hereby has been the conserving effect of the copper and the arsenic acid radicals. Gradually it has become apparent that the copper radical has been more active than the arsenic acid which latter only is given a complementary preserving effect. For this purpose the arsenic acid has not been needed in the amount it heretofore had been used. Other circumstances have had an effect in the 15 same direction. The precipitated arsenic compounds undergo a slow hydrolysis—which phenomenon is not discoverable through short leaching tests—with the consequence that a part of the arsenic acid is separated and leached out. The compound remaining after a long leaching thus contains definitely less arsenic had than 20 the original preservative.

Furthermore, questions of poisoning demand lowest 25 possible content of arsenic. As an example it may here be pointed out that by burning wood which had been treated with arsenic compound the amount of arsenic 30 in the ashes can be alarmingly high.

A still further reason has been that a high amount of 35 arsenic in the preservative has been a source of very serious damage to sleepers in which—as rather common today—weak electric current for signals have been running.

All these circumstances show that the preservative to 40 a higher degree than before ought to be based on copper as conserving agent, and that the amount of arsenic acid has to be reduced as much as possible. Different 45 investigations have shown that the copper content in the impregnating solution normally for full-cell treatment of, for instance, Swedish pine may be kept around 0.3 per cent. If the content of arsenic pentoxide (content of arsenic acid) reaches the same extent as does the copper it is surely enough. It is not excluded that 50 the content of arsenic pentoxide can be reduced to half this amount but hardly below this limit if it shall be possible to make use of the special conserving effect of arsenic. This means that the amount of arsenic pentoxide 55 in relation to the amount of copper is reduced to 1/3 or 1/6 of the amount used in applicant's earlier preservative. A variant of the preservative composition according to this invention, containing no arsenic, has been worked out for use in cases when it is desirable to avoid arsenic as it can be in preservatives for instance for sleepers.

With this the proportions between copper and arsenic pentoxide in the preservative is made clear. Further 60 the preservative must of course be so composed that it can be dissolved in water; it must have a corrosion action on iron or metals; and, after the treatment, it must be precipitated in the wood. The rules for the dissolution is rather simple. One mol CuO is dissolved by 2 mols CrO<sub>3</sub> or by one mol H<sub>2</sub>SO<sub>4</sub>. Even the arsenic acid 65 has some dissolving effect, but it is not of crucial importance in preservatives according to the present invention which now contain compositions comparatively

low in amounts of arsenic acid. For dissolving copper more arsenic is necessary than corresponding to mono-copperarsenate.

The amount of chromic acid needed for the fixation of the copper radical alone, or of copper and arsenic acid, has been investigated by leaching tests on wood treated with solutions of different compositions. Hereby analyses have been carried out on leaching water and on the leached wood in order to ascertain the resistance to leaching of the different ingredients in the preservative. In order to investigate the fixation of the

given: the first figure relates to the amount of arsenic pentoxide, both in hundreds of a per cent. "3/0" thus means that the solution contained 0.30 per cent copper (Cu) and no arsenic pentoxide. "30/45" means 0.30 per cent copper and 0.45 per cent arsenic pentoxide. The first vertical line below each heading means per cent remaining amount of copper in the wood after leaching; the other line means per cent remaining amount of arsenic pentoxide in the wood after leaching. Both lines are given values for increasing chromic acid content.

| 15/0 |      | 15/7,5 |      | 15/15 |      | 15/22,5 |      |
|------|------|--------|------|-------|------|---------|------|
| 92.0 | 92.3 | 88.8   | 89.4 | 76.8  | 94.4 | 60.1    |      |
| 94.7 | 94.4 | 91.8   | 94.4 | 93.8  | 97.3 | 90.9    |      |
| 95.9 | 95.8 | 92.5   | 94.4 | 91.3  | 98.7 | 93.0    |      |
| 96.8 | 95.8 | 95.0   | 93.9 | 95.0  | 99.3 | 93.0    |      |
| 30/0 |      | 30/15  |      | 30/30 |      | 30/45   |      |
| 91.7 | 85.1 | 96.2   | 88.7 | 96.3  | 87.2 | 68.5    | 81.7 |
| 96.4 | 92.2 | 95.9   | 96.4 | 91.2  | 96.9 | 96.3    | 96.0 |
| 97.1 | 92.2 | 92.0   | 97.5 | 92.1  | 98.6 | 97.9    | 98.9 |
| 97.6 | 95.8 | 95.1   | 94.6 | 93.0  | 99.0 | 97.9    | 99.0 |
| 60/0 |      | 60/30  |      | 60/60 |      | 60/90   |      |
| 87.1 | 87.3 | 98.3   | 74.5 | 90.2  | 61.7 | 65.2    |      |
| 96.8 | 91.1 | 99.0   | 91.1 | 98.0  | 91.7 | 98.7    |      |
| 97.9 | 97.9 | 98.4   | 96.0 | 98.0  | 97.6 | 95.0    |      |
| 98.0 | 96.8 | 100.0  | 97.4 | 100.0 | 98.5 | 98.2    |      |

copper radical a certain amount of copper has been introduced into a solution together with different amounts of chromic acid. As a certain amount of chromic acid (as was said above) dissolves only a certain amount of copper oxide (in this experiment carbonate has been used as it reacts faster, and the carbon dioxide evaporates from the acid solutions), a smaller amount of chromic acid has been used than corresponding to bicarbonate of copper (1 mol CuO to 2 mols CrO<sub>3</sub>), the excess of copper having been dissolved in sulphuric acid. A surplus of sulphuric acid has been avoided as this could adversely influence the ensuing fixation.

In the experiments reported hereinbelow the chromic acid contents have amounted to 25, 50, 75 and 100 per cent of the amount corresponding to the formation of soluble bichromate. In the first case 75 per cent of the copper has been dissolved by sulphuric acid; in the second case 50; in the third case 25; while in the fourth case all of the copper was (or, could be) dissolved by the amount of chromic acid present in the composition. In order to make it clear the ingredients of these different solutions can be stated the following way:



In these reported experiments not only the amounts of chromic acid and sulphuric acid have been varied in this way but also different concentrations of the solutions have been tested. The solutions have, further, been tested after addition of arsenic pentoxide in contents amounting to the half and the same amount as the copper content according to what above have been said. In this way a number of solutions have been tested and the results are given in figures meaning the remaining amount in per cent of the different ingredients. As heading in each leaching series two figures have been

From the reported results of these tests it is clear that a comparatively good fixation is obtained when the chromic acid amounts to 25 per cent of the content needed for the formation of bichromate. Twice that amount—i.e., 50 per cent—gives a margin of security.

The corrosion tests show that it is not possible to reduce the amount of the chromic acid drastically without taking serious risks for damages to apparatus; however, if a part of the sulphuric acid is replaced by another acid this problem can be kept under control. Here phosphoric acid has proved to be specially suitable. If all of the sulphuric acid is replaced by phosphoric acid in the different tests no corrosion attack occurs in the above described cases; the same is true if the amount of chromic acid is reduced to 12.5 per cent of the amount corresponding to bichromate. If half the amount of sulphuric acid is replaced by phosphoric acid a content of chromic acid amounting to 50 per cent of the content corresponding to copper bichromate will give a non-corrosive solution. It is here to be observed that one mol sulphuric acid (which dissolves 1 mol copper oxide) in diluted solutions in equivalent—in dissolving effect—to one mol or some more of phosphorous pentoxide. Somewhat more phosphoric acid than that corresponding to mono-copper phosphate thus is necessary for obtaining dissolution.

Sulphuric acid may be replaced by other acids but the possibilities here are very limited. Nitric acid may be used but more corrosion will thereby be obtained. If hydrochloric acid is used an increased risk of corrosion is of course obtained. The introduction of phosphoric acid in the preservative composition causes some changes in the fixation of the ingredients. Thus the fixation of the copper radical is increased while the fixation of the arsenic acid will be decreased to some degree. If half the content of the sulphuric acid is replaced by phosphoric acid a good fixation of both cop-

per- and arsenic- acid radicals is obtained. These facts may be seen from the results of the following figures secured from some leaching tests:

acid and phosphoric acid have been added to the preservative it has been made clear that a less surplus of acid can be tolerated.

| The composition of the solution | Amount chromic acid | Remaining amount of original ingredients after leaching if the below given acids are used: |                 |                                          |      |
|---------------------------------|---------------------|--------------------------------------------------------------------------------------------|-----------------|------------------------------------------|------|
|                                 |                     | Sulphuric acid                                                                             | Phosphoric acid | Mixture of sulphuric and phosphoric acid |      |
| 30/0                            | 25                  | 91.7                                                                                       | —               | 96.3                                     | —    |
|                                 | 50                  | 96.4                                                                                       | —               | 99.0                                     | —    |
| 30/15                           | 25                  | 88.4                                                                                       | 96.2            | 94.0                                     | 71.5 |
|                                 | 50                  | 93.7                                                                                       | 98.6            | 98.0                                     | 90.5 |
| 30/30                           | 25                  | 88.5                                                                                       | 94.6            | 94.3                                     | 59.7 |
|                                 | 50                  | 94.9                                                                                       | 91.2            | 98.3                                     | 89.2 |
| 15/15                           | 25                  | 89.4                                                                                       | 76.8            | 96.5                                     | 53.6 |
|                                 | 50                  | 94.4                                                                                       | 93.8            | 98.1                                     | 85.2 |

It is thus advisable to use a chromic acid content in the preservative amounting at least to 25 per cent of the amount corresponding to the formation of copper bichromate. More than 50 per cent is not necessary for having a good fixation if the copper amount not dissolved by the chromic acid is dissolved to the same and equal parts by sulphuric acid and phosphoric acid. Under these circumstances (1) a good dissolution of the copper radical, (2) a non-corrosive solution and (3) the best possible fixation of the ingredients of the preservative are obtained. As stated above, the content of arsenic pentoxide has to amount to the same or half the copper content.

If the arsenic acid is completely omitted and the preservative is exclusively based on the copper radical the preservative is made in similar way. An amount of chromic acid corresponding to from 25 to 50 per cent of the formation of bichromate may be used. It is desirable to increase the amount of the dissolving acids for ensuring the stability of the solution. Phosphoric acid or a mixture of phosphoric and sulphuric acid, is used and in both cases safety against corrosion is obtained. The sulphuric acid has here no function in increasing the fixation as when arsenic acid is present. For the fixation of the copper radical, on the contrary, phosphoric acid is better. The sulphuric acid may however be included in order to make the preservative easier to dissolve.

Experiments with an increased amount of phosphoric acid  
In the preservative there is no sulphuric acid.

| Amount chromic acid | 30/30                   |      | 30/30 + 0.2 % $H_3PO_4$ |      |      |
|---------------------|-------------------------|------|-------------------------|------|------|
|                     | 25                      | 94.6 | 54.6                    | 90.9 | 50.4 |
|                     | 40                      | 96.3 | 77.5                    | 95.0 | 60.7 |
| Amount chromic acid | 50                      | 97.5 | 86.0                    | 96.5 | 73.4 |
|                     | 30/30 + 0.4 % $H_3PO_4$ |      | 30/30 + 0.6 % $H_3PO_4$ |      |      |
|                     | 25                      | 82.5 | 40.0                    | 75.4 | 31.3 |
| 30                  | 40                      | 92.2 | 66.0                    | 86.3 | 52.7 |
|                     | 50                      | 94.6 | 68.7                    | 92.5 | 64.6 |

Above is presupposed that the smallest possible amount of radicals which can form soluble compounds in the wood after treatment has to be used in the preservative. As radicals composing sodium, potassium and ammonium easily form soluble salts, these radicals have been omitted. The sulphuric acid content has been limited; it is not present to a higher degree than that which is precipitated in the wood in the form of basic salts. The phosphoric acid is fixed very effectively in the amounts used here.

In order further to make the composition of the preservative clear some additional examples will now be given. For one mol  $CuO$  in the preservative one mol  $CrO_3$  is introduced, which dissolves half a mol  $CuO$ . The resulting half part of the copper oxide has as said

Experiments with an increased amount of sulphuric acid

In the preservative there is no phosphoric acid present.

| Amount chromic acid | The composition of the preservatives and remaining amount of original ingredients after leaching: |                      |                      |
|---------------------|---------------------------------------------------------------------------------------------------|----------------------|----------------------|
|                     | 30/30                                                                                             | 30/30+0.1% $H_2SO_4$ | 30/30+0.3% $H_2SO_4$ |
| 25                  | 88.7                                                                                              | 96.3                 | 81.7                 |
| 50                  | 96.4                                                                                              | 91.2                 | 94.0                 |
| 75                  | 97.5                                                                                              | 92.1                 | 97.5                 |
| 100                 | 94.6                                                                                              | 93.0                 | 97.9                 |

30/30+0.1% $H_2SO_4$

30/30+0.3% $H_2SO_4$

Tests have also been carried out in order to establish the influence an excess of acids in the preservative will have on the fixation of different ingredients. From the following leaching tests where a surplus of sulphuric

acid and phosphoric acid that is by  $\frac{1}{4}$  mol  $H_2SO_4$  and  $\frac{1}{4}$   $P_2O_5$ . If the content of arsenic pentoxide amounts to the same content as copper this means an addition of some more

than  $\frac{1}{4}$  mol  $\text{As}_2\text{O}_5$ . The composition of the preservative will thus be the following:



If the different terms in the formula are multiplied by 5 4 the composition can be written in the following way:



This is valid for diluted solutions. When the preservatives are made in the form of solid salts and further have to be resistant to some heating during manufacture, the amounts of chromic acid (and eventually of the sulphuric-phosphoric acids) have to be increased slightly. When the content of arsenic pentoxide is the same as the copper content (a) the chromic acid 10 amount ought to be increased from 50 to 52.5 per cent of the amount corresponding to copper bichromate. If the amount of arsenic pentoxide is half this value, (b) the amount of chromic acid ought to be increased from 15 50 to 60 per cent. In the cases when the arsenic pentoxide is omitted (c) the chromic acid amount ought to be increased to 70 per cent. If in the last case only phosphoric acid is used (and no sulphuric acid) and if so much phosphoric acid is introduced that 50 per cent of the copper corresponds to monophosphate (d) 85 per cent 20 chromic acid ought to be introduced; if the amount of phosphoric acid is increased to twice this amount (e) the amount of chromic acid ought to be 25 65 per cent.

Above described preservatives can be introduced 30 from the following ingredients:

a. 564 parts by weight  $\text{CuO}$

589 parts by weight  $\text{CuSO}_4 \cdot 5 \text{H}_2\text{O}$

991 parts by weight  $\text{CrO}_3$

600 parts by weight  $\text{As}_2\text{O}_5$

546 parts by weight  $\text{H}_3\text{PO}_4$ , 85 per cent

b. 564 parts by weight  $\text{CuO}$

589 parts by weight  $\text{CuSO}_4 \cdot 5 \text{H}_2\text{O}$

- 1133 parts by weight  $\text{CrO}_3$
- 300 parts by weight  $\text{As}_2\text{O}_5$
- 546 parts by weight  $\text{H}_3\text{PO}_4$ , 85 per cent
- c. 564 parts by weight  $\text{CuO}$
- 589 parts by weight  $\text{CuSO}_4 \cdot 5 \text{H}_2\text{O}$
- 1322 parts by weight  $\text{CrO}_3$
- 546 parts by weight  $\text{H}_3\text{PO}_4$ , 85 per cent
- d. 752 parts by weight  $\text{CuO}$
- 1604 parts by weight  $\text{CrO}_3$
- 1092 parts by weight  $\text{H}_3\text{PO}_4$ , 85 per cent
- e. 752 parts by weight  $\text{CuO}$
- 1227 parts by weight  $\text{CrO}_3$
- 2184 parts by weight  $\text{H}_3\text{PO}_4$ , 85 per cent

We claim:

1. A preservative for wood with the following approximate composition

|                                            |                     |
|--------------------------------------------|---------------------|
| $\text{CuO}$                               | 564 parts by weight |
| $\text{CuSO}_4 \cdot 5 \text{H}_2\text{O}$ | 589 parts by weight |
| $\text{CrO}_3$                             | 991 parts by weight |
| $\text{As}_2\text{O}_5$                    | 600 parts by weight |
| $\text{H}_3\text{PO}_4$ , 85 %             | 546 parts by weight |

2. A preservative for wood having the composition in molar relationship



3. A preservative for wood having the following composition:

- 564 parts by weight  $\text{CuO}$
- 589 parts by weight  $\text{CuSO}_4 \cdot 5 \text{H}_2\text{O}$
- 1133 parts by weight  $\text{CrO}_3$
- 300 parts by weight  $\text{As}_2\text{O}_5$
- 546 parts by weight  $\text{H}_3\text{PO}_4$ , 85 per cent.

\* \* \* \* \*